

# United States Patent Office

2,940,851

Patented June 14, 1960

1

**2,940,851**

## SENSITIZATION OF PHOTOGRAPHIC EMULSIONS

**Dorothy J. Beavers, Charles V. Wilson, and James L. Graham, Rochester, N.Y., assignors to Eastman Kodak Company, Rochester, N.Y., a corporation of New Jersey**

No Drawing. Filed Nov. 27, 1957. Ser. No. 699,197

16 Claims. (Cl. 96—60)

This invention relates to the sensitization of photographic silver halide emulsions with certain quaternary ammonium salts, e. g., pyridinium and quinolinium salts.

The sensitization of photographic emulsions with compounds containing quaternary nitrogen atoms has been known for many years as shown by the Carroll U.S. Patent 2,271,623, granted February 3, 1942. A representative quaternary salt sensitizing agent of that patent is the compound ethylene-bis-oxymethylpyridinium perchlorate.

We have discovered certain compounds containing quaternary nitrogen radicals which exhibit improved properties as sensitizing agents for silver halide emulsions. Emulsions containing the compounds of the invention are appreciably more stable than emulsions containing the mentioned quaternary compounds. Accordingly, upon the aging of emulsions containing the new sensitizing agents, less fog is developed and the emulsion speed is maintained. Also, photographic emulsions containing the new quaternary nitrogen compounds maintain their speed over a wider range of development conditions than do emulsions sensitized with previously known alkylene-bis-pyridinium salts such as decamethylene-1,10-bis-pyridinium perchlorate. Thus emulsions containing the latter compound as a sensitizing agent can be expected to lose an appreciable amount of speed when developed with a developing solution of high sulfite content of the order of 100 grams of anhydrous sodium sulfite per liter, whereas the emulsion speed is maintained in such developers when the emulsion is sensitized with the quaternary salts of the present invention.

When the emulsions are sensitized with the quaternary salts of the invention and are used in processes of color photography, that is, in multilayer color films adaptable to the reversal process of color photography, the first development step with the usual Metol-hydroquinone developer produces less fog than when the emulsions are sensitized with other quaternary salts such as that of the above Carroll invention.

It is interesting to note that Howe and Glasset British Patent 566,314 and Vanselow and James PSA Section B, 36-40 (1953), have shown that certain quaternary nitrogen salts such as n-dodecylpyridinium bromide, n-dodecyltriethyl ammonium bromide, etc, are not effective in increasing speed when development is carried out with a p-phenylenediamine as the developing agent such as used in color photography. In fact, it was shown by these workers that development with the p-phenylenediamine developing agent in the presence of the quaternary nitrogen salts retarded the development rate. The quaternary salts of the present invention when employed in the emul-

2

sions as sensitizing agents unexpectedly do not retard development when development is carried out with a *p*-phenylenediamine type developing agent.

5 The quaternary salt sensitizing agents of the invention are bis-quaternary salts having the following general formulas:



and



where Q and Q' represent the same or different organic radicals containing quaternary nitrogen atoms such as trialkyl ammonium salt radicals and cyclammonium salt radicals, e.g., pyridinium salt radicals or quinolinium salt radicals, R and R' represent the same or different radicals, which may be alkylene, such as  $-(\text{CH}_2)_n-$ , and including a carbon chain separated by other atoms such as O or S, e.g.  $-(\text{CH}_2)_n\text{O}(\text{CH}_2)_{n'}$  or  $-(\text{CH}_2)_n-\text{S}-(\text{CH}_2)_{n'}$ , 15 n and n' being integers from about 1 to 10. The total chain length of R and R' must be such that the number of "atoms" in the linear chain joining Q to Q' does not exceed about 30. (The term "atoms" as used herein refers solely to the actual elements that compose the chain 20 and not to any groups that these elements may carry. For example,  $-(\text{CH}_2)_{10}-$  is considered to be a 10-atom chain, the hydrogen atoms being disregarded.



30 is a 12-atom chain, the oxygen and hydrogen atoms being disregarded.) A compound of the above structure wherein in the chain contains 34 atoms has been found not to be useful as a sensitizing agent. Likewise compounds having less than about 14 atoms in the chain are not very useful sensitizing agents, the sensitizing activity of the compounds decreasing rapidly in compounds having less than about 14 or more than about 30 atoms in the linear chain connecting Q to Q'. In a preferred embodiment of the invention, therefore, the compounds contain from about 14 to about 30 atoms in the chain.

35

40

40 from about 14 to about 30 atoms in the chain.



50 When  $n$  equals 2, Formula I above represents a very important class of compounds having the general formula



55 In the above formulas the number of atoms comprising A is limited by the number of atoms in R and R' since as mentioned above, the total number of atoms in the chain connecting Q to Q' must not exceed about 30. Thus in Formula IV, A may contain as many as about 24 atoms  
 60 in a linear chain when R and R' are methylene groups. However, in such compounds where A represents an alkylene group, group A can contain only 2 to about 24 carbon atoms in a linear chain since it has not been possible to synthesize compounds in which A equals a  
 65  $-\text{CH}_2-$  group.

Chains containing carbon, nitrogen, oxygen or sulfur atoms represented by A are as follows:



wherein *n* and *n'* are positive integers of the order of 1 to 10 selected so that the linear chain of atoms between Q and Q' contains from about 14 to about 30 atoms. In the examples hereinafter are provided compounds in which A has been varied as above to obtain very effective sensitizing agents.

Representative bis-quaternary salts having the above formulas are as follows:

I. 4,11-diaza-3,12-dioxotetradecane-1,14 - bis(pyridinium perchlorate)

- II. 10,15-diaza-9,16-dioxotetracosane-1,24 - bis(pyridinium perchlorate)  
III. 12,15-diaza-11,16-dioxohexacosane-1,26 - bis(pyridinium perchlorate)  
IV. 12,19-diaza-11,20-dioxotriaccontane-1,30 - bis(pyridinium perchlorate)  
V. 12,23-diaza-11,24-dioxotetraaccontane - 1,34 - bis(pyridinium perchlorate)  
VI. 7,13-diaza-6,14-dioxo-10-thianonadecane-1,19 - bis(pyridinium perchlorate)  
VII. 7,10,17,20-tetraaza-6,9,18,21 - tetraoxohexacosane-1,26-bis(pyridinium perchlorate)  
VIII. 3-aza-4-oxotetradecane-1,14 - bis(pyridinium perchlorate)  
IX. p-Phenylene-bis(2-aza-3 - oxotridecane pyridinium perchlorate)  
X. 7,18-diaza-6,19-dioxotetracosane-1,24 - bis(trimethyl ammonium p-toluene sulfonate)

A better understanding of the invention can be obtained by consideration of the structural formulas of a number of the compounds of the invention contemplated by the general formulas above.

#### COMPOUND V



#### COMPOUND IX



#### COMPOUND XVI



#### COMPOUND XVII



#### COMPOUND XVIII



#### COMPOUND XIX



II. 4,11-diaza-3,12-dioxotetradecane-1,14-bis(5 - ethyl-2-methyl-pyridinium perchlorate)

III. 3,14-diaza-2,15-dioxohexadecane-1,16 - bis(pyridinium perchlorate)

IV. 4,15-diaza-3,16-dioxooctadecane-1,18 - bis(pyridinium perchlorate)

V. 7,14-diaza-6,15-dioxoeicosane - 1,20 - bis(pyridinium perchlorate)

VI. 7,14-diaza-6,15-dioxoeicosane-1,20-bis(5 - ethyl - α-methyl-pyridinium perchlorate)

VII. 7,14-diaza-6,15-dioxoeicosane-1,20 - bis(pyridinium iodide)

VIII. 7,14-diaza-6,15-dioxoeicosane-1,20 - bis(pyridinium tetraphenyl boron)

IX. 12,13-diaza-11,14-dioxotetracosane-1,24 - bis(pyridinium perchlorate)

X. 7,18-diaza-6,19-dioxotetracosane-1,24 - bis(pyridinium perchlorate)

The compound  $C_5H_5N^+-(CH_2)_{10}CONH(CH_2)_{10}NHCO(CH_2)_{10}-+NC_5H_5$   $2ClO_4$  (XV) containing 34 atoms in the linear chain connecting the quaternary nitrogen atoms is photographically inert and does not impart any appreciable amount of sensitivity to silver halide emulsions.

The sensitizing effect of the representative bis-quaternary nitrogen compound I of the invention having the structure



compared with the following bis-quaternary compound Ir in which the amide linkage is reversed, is interesting.



In compounds I and Ir the same number of atoms are present in the chain separating the quaternary nitrogen atoms yet unexpectedly compound I is superior in regard

to its sensitizing effect upon silver halide as shown by the data in Example 7.

The compounds of the invention having the above general Formulas I, II, III and IV are prepared as indicated in the following flow diagram:

$\omega$ -Bromocaproylchloride, 140 grams (0.66 mole) was dissolved in 500 ml. of dry ether and this solution added through the dropping funnel over a period of one hour, keeping the temperature below 25°. A thick slurry formed immediately and was stirred overnight, then al-



The above diagram shows that the unsymmetrical di-amides can be prepared by reacting the diamine compound consecutively with different  $\omega$ -halo acids, then acid halides. The symmetrical amides are prepared by reacting two moles of the  $\omega$ -halo acid or acid chloride with the desired diamine in a single step followed by the quaternization step. For photographic purposes, the quaternary nitrogen compounds obtained as the halide salts are preferably converted to inert salts such as the perchlorate as illustrated in the syntheses hereafter. In the above flow diagram X represents a halogen atom, e.g., chlorine, bromine or iodine or alkyl or aryl sulfonate ester; R, R', A and n, Q and Q' have the significance given above. Representative bis-quaternary salts of this type are synthesized as follows:

#### COMPOUND VI

##### $\omega$ -Bromocaproic acid

$\omega$ -Bromocapronitrile, 202 g. (1.15 mole), 350 ml. of 48% hydrobromic acid and 350 ml. of glacial acetic acid were refluxed vigorously for fifteen hours. The product was diluted with 500 ml. of ice water and extracted three times with 500 ml. portions of ether. The solvent was removed on the steam bath and the residue stripped under reduced pressure to remove any acetic acid which may have been extracted along with the product. The 216 g. of crude oil was fractionated under vacuum to yield 181 g. (81.5% yield) of a colorless oil, B.P. 120-140°/1.2 mm. which solidified to white platelets M.P. 27-29°.

##### $\omega$ -Bromocaproylchloride

To 250 ml. of dry benzene was added 280 g. (1.44 mole) of  $\omega$ -bromocaproic acid. The solution was stirred while 230 g. of oxalyl chloride was added over a period of thirty minutes. A vigorous evolution of hydrogen chloride took place although no temperature rise was evident. The solution was allowed to stand one hour at room temperature, then heated to 60° for two hours. The solvent was removed at 60° under the aspirator. The pale yellow oil weighing 323 g. was fractionated through a 6" "Vigreau" column. A pale yellow oil with an acid chloride odor weighing 291 g. (95%) was collected at 95-102°/1 mm.

##### 7,14-diaza-6,15-dioxoeicosane-1,20-dibromide

To a 5 liter flask equipped with stirrer, dropping funnel and condenser was added three liters of dry ether. Thirty-eight grams (0.33 mole) of freshly distilled hexamethylenediamine and 73 grams (0.73 mole) of triethylamine were added to the flask giving a clear solution.

lowed to stand for twenty-four hours at room temperature. The thick white slurry was filtered as dry as possible with suction and the remaining traces of ether removed in the vacuum oven at room temperature. The 30 finely divided white powder was vigorously slurried in 2 liters of ice water for fifteen minutes, then filtered. The filter cake was reslurried with ether, filtered, and dried at room temperature in the vacuum oven giving 152 grams (98% yield) of cream-colored solid of M.P. 35 110.5-112°. If the melting point of the solid is much lower, the dibromide is dissolved in a minimum of methanol, filtered, ether added to the cloudpoint, and the solution chilled in a Dry Ice acetone bath. With 40 vigorous scratching a crystalline solid of excellent melting point is obtained. The analytical sample was obtained as white needles from acetone and melted at 110-112.5°.

*Analysis.*—Calc. for C<sub>18</sub>H<sub>34</sub>Br<sub>2</sub>N<sub>2</sub>O<sub>2</sub>: C, 46.0; H, 7.2; N, 6.0; Br, 34.0. Found: C, 45.8; H, 7.0; N, 6.1; Br, 45 33.7.

##### 7,14-diaza-6,15-dioxoeicosane-1,20-bis(pyridinium perchlorate)

One hundred thirty g. of 7,14-diaza-6,15-dioxoeicosane-1,20-dibromide was added to 700 ml. of pyridine and the mixture heated to reflux for 2 hours. (The solution began precipitating the quaternary salt as an oil after the first 20 minutes of refluxing.) The mixture was cooled, the excess pyridine decanted and the dark orange oil slurried with ether several times, the ether being decanted each time. The syrup was dissolved in a small amount of methanol, and dry ether added until no more oil precipitated. The ether was decanted and the trace of solvent removed on the steam bath under 55 vacuum leaving 177 g. of a dark orange oil which contained no pyridine odor.

The oil was dissolved in 500 ml. of methanol in a flask equipped with an efficient stirrer. A solution of 95.0 g. (0.68 mole) of sodium perchlorate monohydrate in 500 ml. of acetone was added and the thick slurry heated for one-half hour on the steam bath. The sodium bromide which had precipitated was filtered off and the solution concentrated to about a 300 ml. volume. Acetone, 300 ml., was added and the mixture heated. The sodium bromide which precipitated was filtered off. The solution was chilled in a Dry-Ice acetone bath and with vigorous scratching, dry ether was slowly added to the cloud point. The scratching was continued until a solid precipitate appeared, or if an oil appeared, the 65 excess ether was removed, the solution chilled and the

ether added again with scratching. (The initial crystallization may take some time.) A sticky cream colored solid was filtered off. It was redissolved in a minimum of methanol, the product chilled, and ether slowly added with scratching. (A seed from the initial crystallization will hasten the second crystallization.) A cream-colored solid weighing 139 g. (74%) and melting at 54-57° was obtained. This product was recrystallized from methanol-ether in the same way, giving a semi-crystalline white solid weighing 117 g. (64.5%) with M.P. 60-63°. Samples of this pyridinium perchlorate melting as low as 50° have proven satisfactory as photographic supersensitizers.

The analytical sample was obtained from methanol-ether as a white semi-crystalline solid, M.P. 60.5-63.5°.

*Analysis.*—Calc. for  $C_{28}H_{44}Cl_2N_4O_10$ : C, 50.4; H, 6.6; N, 8.4; Cl, 10.7. Found: C, 50.3; H, 6.2; N, 8.5; Cl, 10.3.

#### COMPOUND X

##### 1,10-diaminodecane

A twelve liter flask was equipped with a powerful stirrer, an efficient condenser, and a powder funnel. Eight liters of dry ether were added to the flask and the apparatus swept out with a stream of nitrogen. Granular lithium aluminum hydride, 100 g. (2.6 mole) was added through the powder funnel under a nitrogen atmosphere. The funnel was replaced by a dropping funnel and a solution of 342 g. (2.6 mole) of anhydrous aluminum chloride in one liter of dry ether was added as rapidly as possible and the resulting slurry stirred for 15 minutes.

A solution of 213 g. (1.3 mole) of sebaconitrile in 250 ml. of dry ether was now added through the dropping funnel rapidly enough to cause a noticeable reflux. About one hour is necessary for the complete addition of the nitrile. The grey mixture was refluxed for two hours, then stirred at room temperature overnight.

The lithium-aluminum hydride-diamine complex was decomposed by slowly adding a solution of 250 g. of sodium hydroxide in one-liter of water through the dropping funnel while allowing most of the ether to escape. One pound of sodium chloride was added to the resulting grey liquid slurry and the mixture stirred vigorously with two 2 l. portions of hot benzene, the benzene layers being decanted each time. The benzene was removed from the extracts on the steam bath under vacuum leaving 129 g. of a colorless oil which solidified to a white crystalline mass of decamethylenediamine of M.P. 55-57.5°. The diamine should be protected from the atmosphere as it readily picks up carbon dioxide from the air forming the dicarbonate salt.

The remaining slurry was extracted continuously with benzene in a liquid-liquid extractor for sixteen hours giving an additional 44.5 g. of diamine possessing a slight yellow color with M.P. 53-56°. The overall yield of 1,10-diaminodecane suitable for further reaction is 173.5 g. (78%).

##### 7,18-diaza-6,19-dioxotetracosane-1,24-dibromide

One hundred one grams (0.59 mole) of 1,10-diaminodecane was dissolved in 500 ml. of dry benzene. This solution was added to a 5 l. flask equipped with an efficient stirring motor, a dropping funnel and condenser. Triethylamine, 130 g. (1.29 mole) was added to the solution followed by the addition of 3 liters of dry ether. A solution of 250 g. (1.17 mole) of  $\omega$ -bromocaproyl chloride in 200 ml. of dry ether was added to the turbid solution over a period of one hour, keeping the temperature of the slurry below 25°. The thick slurry was stirred at room temperature for four hours, then allowed to stand for twenty-four hours. The slurry was filtered as dry as possible with suction, washed with ether and dried in the vacuum oven at room temperature. The finely divided solid was added to 2 liters of ice water and rapidly agitated for 15 minutes. The slurry was filtered with suction, slurred in ether, filtered again, and the white crys-

talline solid dried in the vacuum oven. The dibromide weighed 285 g. (92%) and had a M.P. of 103.5-106.5°. Yields of 85-98% of product have been obtained in this reaction.

The analytical sample (from ethanol) melted at 105.5-107.5.

*Analysis.*—Calc. for  $C_{22}H_{42}Br_2N_2O_2$ : C, 50.2; H, 7.9; N, 5.3; Br, 30.4. Found: C, 51.0; H, 8.0; N, 5.5; Br, 30.2.

##### 7,18-diaza-6,19-dioxotetracosane-1,24-bis(pyridinium perchlorate)

To a 2-l. flask equipped with condenser was added 285 g. (0.54 mole) of 7,18-diaza-6,19-dioxotetracosane-1,24-dibromide and 1500 ml. of dry pyridine. The solution was heated to reflux for one and one-half hours, although the quaternary salt precipitated out as an orange oil after the first fifteen minutes. The mixture was chilled, the excess pyridine decanted, and the golden syrup slurred several times with ether, the ether being decanted. The oil was finally dissolved in a minimum of methanol, and ether added until no more oil precipitated from the solution. The product was chilled, the ether decanted, and the remaining traces of solvent removed on the steam bath under vacuum leaving a viscous orange oil with no pyridine odor.

The oil was dissolved in 500 ml. of methanol and with efficient stirring a solution of 182 g. (1.30 mole; 20% excess) of sodium perchlorate monohydrate in

30 1600 ml. of acetone was added. The precipitating sodium bromide formed a thick slurry. The mixture was concentrated on the steam bath to one-half the original volume and the slurry filtered with suction. The solution was now concentrated to about 400 ml. and this sticky residue heated and slurred with one l. of acetone. The sodium bromide which had precipitated was filtered off and the solution concentrated to  $\frac{1}{2}$  l. Two hundred ml. of methanol was added, and the solution chilled in a Dry Ice acetone bath. Ether was slowly added, with vigorous scratching until the cloud point was reached, or until a solid began precipitating from solution. If an oil formed first, vigorous scratching of the oil usually resulted in the oil solidifying; or ether could be removed, the solution chilled again, and the process repeated. The sticky cream colored solid melting at 60-63° was dissolved in a minimum of methanol, chilled in a Dry Ice-acetone bath and ether slowly added with scratching until a solid began precipitating from solution. The white semi-crystalline solid melted at 64-66.5°. Another recrystallization of the solid from methanol-ether in the same manner raised the melting point to 67-70°. The cream-colored solid weighed 338 g. (86.5%).

The analytical sample when recrystallized several times from methanol-ether melted at 72-75°.

*Analysis.*—Calc. for  $C_{32}H_{54}Cl_2N_4O_10$ : C, 53.1; H, 7.2; N, 7.8; Cl, 9.8. Found: C, 52.9; H, 7.4; N, 7.9; Cl, 9.5.

#### COMPOUND XI

##### 10,15-diaza-9,16-dioxotetracosane-1,24-dibromide

A solution of 30.8 g. (0.19 mole) of 1,4-diaminobutane dihydrochloride in 250 ml. of water was added to a 1 l. flask equipped with stirrer and dropping funnel. A solution of 38.4 g. (0.96 mole) of sodium hydroxide in 200 ml. of water was added and the mixture chilled below 10°. The  $\omega$ -bromopelargonyl chloride (103 g., 0.38 mole) was added through the dropping funnel at such a rate that the temperature of the slurry never rose above 10°. After stirring at 0°-10° for two hours, the white solid was filtered as dry as possible, then washed with ether. The crude white solid, recrystallized from methanol-ether, gave 67.5 g. (67.5 percent) of dibromide melting at 116.5-119°.

##### 10,15-diaza-9,16-dioxotetracosane-1,24-bis(pyridinium perchlorate)

A solution of 67.5 g. (0.129 mole) of 10,15-diaza-

9,16-dioxotetracosane-1,24-dibromide in 275 ml. of dry pyridine was refluxed for two hours. An oil precipitated from solution after the first half hour. The pyridine was removed completely from the product on the steam bath under vacuum. The residue was dissolved in 300 ml. of methanol and added to a solution of 43.0 g. (0.31 mole) of sodium perchlorate monohydrate in 300 ml. of methanol with vigorous stirring. After heating for one hour while concentrating the solution to one-half the original volume, the precipitated sodium bromide was filtered off. This procedure was repeated until sodium bromide no longer precipitated.

The solution was chilled in Dry Ice-acetone and ether slowly added with intense scratching. The solvent was decanted from the sticky solid that separated. This semi-solid was dissolved in methanol, chilled in a Dry Ice-acetone bath, and the treatment with ether repeated. A solid melting at 65-75° (cloudy) was obtained. Recrystallization of this solid from methanol-ether in the same manner gave 71 g. (72.5 percent) of product melting at 76-78° with preliminary softening at 72°.

An analytical sample was obtained from methanol upon chilling in a Dry Ice-acetone bath, melting point 80-82.5°.

*Analysis.*—Calc. for  $C_{32}H_{52}N_4O_1Cl_2$ : C, 53.1; H, 7.2; N, 7.8; Cl, 9.8. Found: C, 53.6; H, 7.5; N, 7.8; Cl, 9.2.

### COMPOUND XVII

#### *Ethyl N- $\omega$ -bromocaproylglycinate*

A mixture of 19.5 g. (0.10 mole) of  $\omega$ -bromocaprylic acid and 12.9 g. (0.10 mole) of carbethoxymethyl isocyanate (mildly exothermic) was heated on the steam bath under anhydrous conditions for six hours. An evolution of carbon dioxide was evident during the reaction. A yellow oil resulted which was dissolved in 50 ml. of dry ether, cooled, and petroleum ether added slowly. A white crystalline solid weighing 18.4 g. (65.7 percent) and melting at 46.5-48.5° was filtered from the mixture.

The analytical sample of the ester was obtained as matted white needles from ether-petroleum ether, melting point 46.5-48.5°.

*Analysis.*—Calc. for  $C_{10}H_{18}O_3$  NBr: C, 42.9; H, 6.4; N, 5.0; Br, 28.6. Found: C, 42.9; H, 6.3; N, 5.2; Br, 28.7.

#### *N- $\omega$ -bromocaproylglycine*

*N- $\omega$ -bromocaproylglycine* ethyl ester was prepared as above from 52 g. (0.27 mole) of  $\omega$ -bromocaproylglycine and 34.4 g. carbethoxymethyl isocyanate (0.27 mole) and used without further purification for the hydrolysis.

The pale yellow ester was dissolved in 100 ml. methanol and hydrolyzed by slowly adding a solution of 21.2 g. (0.53 mole) sodium hydroxide in 22 ml. of water. The temperature was not allowed to rise above 50° during the addition. After one-half hour, the solution was poured into a large volume of ether, precipitating the sodium salt. The white solid weighed 86 g. (contained some NaOH) and melted cloudy at 174-177°.

Forty grams of the above salt was dissolved in 20 ml. of water and neutralized to a pH of 3 with 1:1 hydrochloric acid. The mixture was saturated with sodium chloride and then extracted several times with warm benzene and ethyl acetate. The extracts were dried over sodium sulfate, and the solvent removed, leaving 21.0 g. (57 percent) of the substituted glycine as an oil. The acid is extremely difficult to extract, being only slightly soluble in benzene and ethyl acetate, almost completely insoluble in ether, and fairly soluble in water, even when the aqueous solution has been saturated with sodium chloride.

An analytical sample of the acid was obtained from methanol-petroleum ether and melted at 69.5-70.5°.

*Analysis.*—Calc. for  $C_8H_{14}NO_3$  Br: C, 38.1; H, 5.6; N, 5.6; Br, 31.8. Found: C, 38.9; H, 5.4; N, 4.7; Br, 30.8.

#### 7,10,17,20 - tetraza - 6,9,18,21 - tetraoxohexacosane-1,26-dibromide

Seven grams (0.042 mole) of hexamethylene diisocyanate in 50 ml. of dry benzene was added to 21 g. (0.083 mole) of  $N-\omega$ -bromocaproylglycine in 100 ml. dry benzene. The solution was refluxed vigorously. After ten hours, the cream-colored solid that gradually separated in the reaction mixture was collected on a filter and dried; yield, 16.3 g., melting point 150-160°.

10 The powder was dissolved in 250 ml. of methanol, filtered, and crystallized; melting point 165-175°, softening at 150°. A recrystallization from ethanol gave 10.3 g. (41 percent) of white powder of melting point 175-178° (softens at 160°).

15 *Analysis.*—Calc. for  $C_{22}H_{40}N_4O_4Br_2$ : C, 45.2; H, 6.8; N, 9.6; Br, 27.4. Found: C, 47.6; H, 7.0; N, 10.3; Br, 20.4.

#### 7,10,17,20 - tetraza - 6,9,18,21 - tetraoxohexacosane-1,26-bis(pyridinium perchlorate)

20 Four grams (0.0069 mole) of the dibromide just above was refluxed vigorously with 25 ml. of pyridine and 25 ml. of ethanol for three hours. The ethanol and pyridine were removed completely on the steam bath under vacuum, leaving a yellow water-soluble gum.

25 The gum was dissolved in 25 ml. of methanol and a solution of 2.1 g. (0.015 mole) of sodium perchlorate monohydrate in 50 ml. of acetone added. The solution was heated until only 20 ml. of a slurry remained and the precipitated sodium bromide filtered off.

30 The product was precipitated from ethanol-ether as a sticky white solid when chilled in a Dry Ice-acetone bath. This sticky solid was recrystallized from methanol-ether as a wax which when triturated with ether turned to 2.0 g. of a white solid of melting point 90-100° dec. (38 percent).

35 *Analysis.*—Calc. for  $C_{32}H_{60}N_6O_1Cl_2$ : C, 49.2; H, 6.4; N, 10.8; Cl, 9.1. Found: C, 47.7; H, 6.4; N, 10.7; Cl, 8.1.

40 The alternate procedure of preparing quaternary salts of bis-amides from the  $\alpha,\omega$ -dihalide



45 in the flow diagram is illustrated by the following synthesis.

### COMPOUND XX

#### 7,18 - diaza - 6,19 - dioxotetracosane - 1,24 - bis(dimethylamine hydrobromide)

50 A mixture of 21.0 g. (0.04 mole) of 7,18-diaza-6,19-dioxotetracosane-1,24-dibromide (prepared as above), 75 ml. of dimethylamine, and 250 ml. of ethanol was heated in a Paar bomb for 16 hours on the steam bath, then allowed to cool slowly to room temperature. The 5 g. of crystalline solid which precipitated was filtered off and identified as starting dibromide.

55 The orange filtrate was concentrated to about 50 ml. and ether slowly added while chilling in a Dry-Ice-acetone bath. A water-soluble tan solid (15.3 g., 62 percent yield), M.P. 118.5-123.5° was obtained.

60 A solution of 11.4 g. (0.0185 mole) of 7,18-diaza-6,19-dioxotetracosane-1,24-bis(dimethylamine hydrobromide), in 50 ml. of water was added to a solution of 7.7 g. (0.056 mole) of potassium carbonate in 50 ml. of water. Chunks of ice were added until no more amine precipitated and the solid was filtered off, M.P. 108-110°, wt. 7.0 g. (83.5 percent). The amine was dissolved in acetone, filtered, and the solution chilled in a Dry-Ice-acetone bath while slowly adding ether. A white crystalline solid (4 g. 48 percent), M.P. 110-111.5° was obtained.

65 *Analysis.*—Calc. for  $C_{28}H_{54}N_4O_2$ : C, 68.8; H, 11.9; N, 12.3. Found: C, 68.0; H, 11.5; N, 12.2.

70 Twenty ml. of ethanol, 2.1 g. (0.011 mole) of methyl p-toluenesulfonate, and 2.3 g. (0.005 mole) of the above

bisamine were refluxed on the steam bath for two hours. The mixture was concentrated to about a 15-ml. volume and ether added. A white solid precipitated immediately, weighing 4.0 g. (98 percent yield) M.P. 182-184° C.; softens 175° C.

After two recrystallizations from methanol-ether, a beautiful white crystalline hygroscopic solid was obtained, 3.8 g., M.P. 188-190°. The analysis indicates that the salt may contain water of crystallization, or solvent of crystallization.

*Analysis.*—Calc. for  $C_{42}H_{74}N_4O_8S_2$ : C, 61.0; H, 9.0; N, 6.8; S, 7.8. Found: C, 56.6; H, 8.8; N, 7.5; S, 8.6.

The preparation of a monoamide as indicated in the flow diagram above is carried out as follows:

### COMPOUND XVIII

#### 3-azo-4-oxotetradecane-1,14-dibromide

Fifteen grams (0.073 mole) of 2-bromoethylamine hydrobromide and 8.4 g. (0.21 mole) of sodium hydroxide were dissolved in 75 ml. of ice water. Keeping the temperature at 0°, 20.8 g. (0.073 mole) of  $\omega$ -bromoundecanoyl chloride was slowly added through a dropping funnel. After the complete addition of the chloride, the slurry was stirred at room temperature for 1½ hours, then filtered with suction.

An analytically pure product (16 g., 59 percent) was obtained by recrystallization from alcohol, M.P. 113-115°.

*Analysis.*—Calc. for  $C_{13}H_{25}Br_2NO \cdot H_2O$ : C, 40.0; H, 6.9; N, 3.6; Br, 41.0. Found: C, 40.2; H, 6.8; N, 3.6; Br, 40.1.

#### 3-aza-4-oxotetradecane-1,14-bis(pyridinium perchlorate)

Twenty-five ml. of dry pyridine and 5.0 g. (0.013 mole) of 3-aza-4-oxotetradecane-1,14-dibromide were heated at reflux for three hours. The excess pyridine was removed and the oil slurried several times with ether to remove traces of pyridine.

The residual oil was dissolved in 25 ml. of methanol, and a solution of 4.6 g. of sodium perchlorate monohydrate in 25 ml. of acetone was added. The solution was concentrated on the steam bath to one-half the volume and the inorganic salt filtered off. This procedure was carried out until no more sodium bromide precipitated upon concentrating the oil. The water-soluble oil would not crystallize after several attempts; therefore, it was isolated as a pale yellow oil (4 g.).

The other bis-quaternary compounds of the invention may be prepared in a similar manner by selection of the appropriate diamine for reaction with the appropriate organic acid or organic acid halide.

The following examples illustrate the use of the bis-quaternary salts of the invention in photographic emulsions:

#### EXAMPLE 1

A high-speed bromoiodide emulsion was prepared, chemically sensitized with sulfur and gold compounds and optically sensitized with a cyanine dye. The amounts of the bis-quaternary nitrogen compounds shown in Table I below were added to samples of the emulsion alone and together with an azaindene stabilizing agent. The emulsion samples were then coated, exposed on a sensitometer and developed for 5 minutes at 68° F. in the developer given below. The speed, gamma and fog values obtained by sensitometric evaluation of the developed samples are also shown in the table. The speed values shown are expressed at 100 (1-log E) where E is the exposure in meter candle seconds required to produce in the emulsion a density of 0.3 above fog.

|                          |       |      |    |
|--------------------------|-------|------|----|
| Water                    | cc    | 500  | 70 |
| Elon                     | grams | 2.5  |    |
| Sodium sulfite anhydrous | do    | 30.0 |    |
| Hydroquinone             | do    | 2.5  |    |
| Sodium metaperborate     | do    | 10.0 |    |
| Potassium bromide        | do    | 0.5  | 75 |

TABLE I

| Number | Feature                                                                               | Speed | $\gamma$ | Fog  |
|--------|---------------------------------------------------------------------------------------|-------|----------|------|
| 5 932  | Control                                                                               | 318   | 1.12     | 0.16 |
| 930    | 4,11-Di-3,12-dioxotetradecane-1,14-bis(pyridinium perchlorate) (I) 0.75 g./mol./AgX.  | 328   | 1.23     | .18  |
| 927    | 8,14-Di-2,15-dioxohexadecane-1,16-bis(pyridinium perchlorate) (III) 0.75 g./mol./AgX. | 328   | 1.10     | .20  |
| 10 933 | 4-Hydroxy-6-methyl-1,3,3a,7-tetraazaindene (XXX) 3.0 g./mol./AgX.                     | 324   | 1.17     | .15  |
| 944    | (XXX) 3.0 g./mol.+(I) 0.75 g./mol.                                                    | 327   | 1.21     | .17  |
| 945    | (XXX) 3.0 g./mol.+(I) 2.25 g./mol.                                                    | 330   | 1.10     | .17  |
| 936    | (XXX) 3.0 g./mol.+(III) 0.75 g./mol.                                                  | 328   | 1.00     | .18  |
| 937    | (XXX) 3.0 g./mol.+(III) 2.25 g./mol.                                                  | 330   | .97      | .20  |

#### EXAMPLE 2

15 An emulsion was provided as in Example 1 and the additions shown in Table II were made to samples of the emulsion. Sensitometric evaluation made as described in Example 1 gave the results shown in the table.

TABLE II

| Number | Feature                                                                           | Speed | $\gamma$ | Fog  |
|--------|-----------------------------------------------------------------------------------|-------|----------|------|
| 115    | Control                                                                           | 310   | 1.17     | 0.15 |
| 112    | 7,14-Di-6,15-dioxoicosane-1,20-bis(pyridinium perchlorate) (V) 0.75 g./mol.       | 334   | 1.20     | .22  |
| 25 113 | 7,18-Di-6,19-dioxotetraicosane-1,24-bis(pyridinium perchlorate) (VI) 0.75 g./mol. | 331   | 1.07     | .25  |
| 116    | 4-Hydroxy-6-methyl-1,3,3a,7-tetraazaindene (XXX) 3.0 g./mol.                      | 316   | 1.11     | .15  |
| 123    | (XXX) 3.0 g./mol.+(V) 0.75 g./mol.                                                | 337   | 1.20     | .18  |
| 124    | (XXX) 3.0 g./mol.+(V) 2.25 g./mol.                                                | 343   | 1.17     | .19  |
| 30 125 | (XXX) 3.0 g./mol.+(VI) 0.75 g./mol.                                               | 337   | 1.07     | .21  |
| 126    | (XXX) 3.0 g./mol.+(VI) 2.25 g./mol.                                               | 346   | 1.07     | .21  |

#### EXAMPLE 3

35 An emulsion was provided as in Example 1 but with the addition to samples of the emulsion of compounds IX and XI, as shown in Table III. Processing was carried out as in Example 1 for evaluating the emulsion sensitivity and other characteristics of the emulsion.

TABLE III

| Number | Feature                                                                             | Speed | $\gamma$ | Fog |
|--------|-------------------------------------------------------------------------------------|-------|----------|-----|
| 537    | Control                                                                             | 314   | 1.08     | .17 |
| 542    | 12,13-Di-11,14-dioxotetraicosane-1,24-bis(pyridinium perchlorate) (IX) 0.75 g./mol. | 340   | 1.01     | .32 |
| 543    | 10,15-Di-9,16-dioxotetraicosane-1,24-bis(pyridinium perchlorate) (XI) 0.75 g./mol.  | 337   | 1.24     | .30 |
| 546    | 4-Hydroxy-6-methyl-1,3,3a,7-tetraazaindene (XXX) 3.0 g./mol.                        | 326   | 1.36     | .18 |
| 554    | (XXX) 3.0 g./mol.+(IX) 0.75 g./mol.                                                 | 347   | 1.08     | .26 |
| 555    | (XXX) 3.0 g./mol.+(V) 2.25 g./mol.                                                  | 347   | 1.02     | .30 |
| 556    | (XXX) 3.0 g./mol.+(XI) 0.75 g./mol.                                                 | 345   | 1.24     | .25 |
| 557    | (XXX) 3.0 g./mol.+(XI) 2.25 g./mol.                                                 | 353   | 1.26     | .25 |

#### EXAMPLE 4

55 An emulsion was prepared and tested as in Example 1 using the bis-quaternary compounds shown in Table IV. The data of this example compares the diamide compounds VI and II with the tetramide compound XVII alone and in the presence of the azaindene stabilizing agent XXX.

TABLE IV

| Number | Feature                                                                                           | Speed | $\gamma$ | Fog  |
|--------|---------------------------------------------------------------------------------------------------|-------|----------|------|
| 1977   | Control                                                                                           | 308   | 1.30     | 0.17 |
| 1982   | 7,14-Di-6,15-dioxoicosane-1,20-bis(5-ethyl-2-methyl-pyridinium perchlorate) (VII) 0.75 g./mol.    | 327   | 1.06     | .24  |
| 1983   | 4,11-Di-3,12-dioxotetradecane-1,14-bis(5-ethyl-2-methyl-pyridinium perchlorate) (II) 0.75 g./mol. | 325   | 1.32     | .21  |
| 1985   | 7,10,17,20-Tetra-6,9,18,21-tetraoxo-1,26-bis(pyridinium perchlorate) (XVII) 0.75 g./mol.          | 322   | 1.26     | .20  |
| 2005   | 4-Hydroxy-6-methyl-1,3,3a,7-tetraazaindene (XXX) 3.0 g./mol.                                      | 317   | 1.35     | .14  |
| 1994   | (XXX) 3.0 g./mol.+(VII) 0.75 g./mol.                                                              | 325   | 1.19     | .19  |
| 1995   | (XXX) 3.0 g./mol.+(VI) 2.25 g./mol.                                                               | 329   | 1.23     | .21  |
| 1997   | (XXX) 3.0 g./mol.+(II) 0.75 g./mol.                                                               | 326   | 1.27     | .17  |
| 1998   | (XXX) 3.0 g./mol.+(II) 2.25 g./mol.                                                               | 325   | 1.21     | .19  |
| 2003   | (XXX) 3.0 g./mol.+(XVII) 0.75 g./mol.                                                             | 328   | 1.35     | .17  |
| 2004   | (XXX) 3.0 g./mol.+(XVII) 2.25 g./mol.                                                             | 329   | 1.30     | .18  |

13  
EXAMPLE 5

A fast bromoiodide emulsion was chemically sensitized with sulfur and gold compounds and optically sensitized with a combination of cyanine dyes. In addition, 3.0 grams per mole of silver halide of 4-hydroxy-6-methyl-1,3,3a,7-tetrazaindene and 0.75 gram per mole of silver halide of a polyethylene oxide of average molecular weight 1500 were added. The amounts of the alkylene bis-pyridinium salt and compounds X and XI shown in Table V were then added and the emulsions coated. Testing was carried out as in Example 1 upon the freshly coated emulsion samples and other samples of each emulsion were incubated for 1 week at 120° F. and 50 percent relative humidity. Still other samples of each emulsion were stored under room conditions 78° F. Keeping" and developed with the same developing solution given in Example 1 with the result shown in Table V. Consideration of the "Fog" data in the table shows

## 14

fixation, silver bleaching and final fixation. Color Process 1 was carried out at 75° F. as follows:

- (1) Negative development—10 minutes
- (2) Reversal flash exposure
- (3) Color development—15 minutes
- (4) Silver bleaching—8 minutes
- (5) Fixing—3 minutes

The negative developer had the following composition:

|    |                                              |        |      |
|----|----------------------------------------------|--------|------|
| 10 | Water, 90° F. (32° C.)                       | liters | 1.0  |
|    | Sodium hexametaphosphate                     | grams  | 2.0  |
| 5  | N-methyl p-aminophenol sulfate               | do     | 6.0  |
|    | Sodium sulfite, desiccated                   | do     | 50.0 |
| 15 | Hydroquinone                                 | do     | 6.0  |
|    | Sodium carbonate, monohydrated               | do     | 35.0 |
|    | Potassium bromide                            | do     | 2.0  |
|    | Sodium thiocyanate                           | do     | 1.5  |
|    | 0.5% solution (6-nitrobenzimidazole nitrate) | cc     | 12.0 |
|    | 0.1% solution of potassium iodide            | cc     | 10.0 |

TABLE V

| Number | Feature                                                                                 | Fresh Tests |      |      | Incubation,<br>1 wk., 120° F. |      |      | 3 Months, 78° F.,<br>Keeping |      |      |
|--------|-----------------------------------------------------------------------------------------|-------------|------|------|-------------------------------|------|------|------------------------------|------|------|
|        |                                                                                         | Sp.         | γ    | Fog  | Sp.                           | γ    | Fog  | Sp.                          | γ    | Fog  |
| 7810   | Control                                                                                 | 342         | 1.12 | 0.15 | 343                           | 1.01 | 0.16 | 337                          | 1.05 | 0.16 |
| 7820   | Hexadecamethylene-1,16-bis(pyridinium perchlorate) 0.15 g./mol AgX.                     | 356         | 1.10 | .24  | 359                           | 1.10 | .22  | 353                          | 1.20 | .20  |
| 7821   | Hexadecamethylene-1,16-bis(pyridinium perchlorate) 0.3 g./mol AgX.                      | 356         | 1.24 | .30  | 359                           | 1.02 | .34  | 359                          | 1.23 | .26  |
| 7822   | Hexadecamethylene-1,16-bis(pyridinium perchlorate) 0.6 g./mol AgX.                      | 355         | 1.17 | .29  | 345                           | .90  | .48  | 356                          | 1.23 | .31  |
| 7826   | 7,18-Diaza-6,19-dioxotetacosane-1,24-bis-(pyridinium perchlorate) (X) 0.45 g./mol AgX.  | 352         | 1.09 | .19  | 364                           | 1.01 | .19  | 351                          | 1.27 | .19  |
| 7827   | 7,18-Diaza-6,19-dioxotetacosane-1,24-bis-(pyridinium perchlorate) (X) 0.75 g./mol AgX.  | 358         | 1.14 | .20  | 362                           | 1.20 | .20  | 353                          | 1.32 | .19  |
| 7828   | 7,18-Diaza-6,19-dioxotetacosane-1,24-bis-(pyridinium perchlorate) (X) 1.2 g./mol AgX.   | 357         | 1.33 | .23  | 362                           | 1.18 | .22  | 354                          | 1.25 | .20  |
| 7839   | 10,15-Diaza-9,16-dioxotetacosane-1,24-bis-(pyridinium perchlorate) (X) 0.45 g./mol AgX. | 352         | 1.22 | .18  | 352                           | 1.25 | .20  | 350                          | 1.18 | .17  |
| 7840   | 10,15-Diaza-9,16-dioxotetacosane-1,24-bis-(pyridinium perchlorate) (X) 0.75 g./mol AgX. | 357         | 1.25 | .19  | 359                           | 1.15 | .19  | 354                          | 1.33 | .17  |
| 7841   | 10,15-Diaza-9,16-dioxotetacosane-1,24-bis-(pyridinium perchlorate) (X) 1.2 g./mol AgX.  | 358         | 1.38 | .19  | 361                           | 1.20 | .20  | 356                          | 1.28 | .17  |

that the emulsions containing compounds X and XI of the invention were more stable than the emulsions containing the alkylene bis-pyridinium compound of the prior art.

## EXAMPLE 6

The use of the bis-quaternary salts of the invention in color photography is illustrated in this example.

A sulfur and gold sensitized gelatino silver bromoiodide emulsion was ripened to maximum sensitivity. To this emulsion was added an optical sensitizing dye that extended the light sensitivity to 6000-7000 A. and a hydrophobic cyan color former suitably dispersed in a high boiling organic solvent. A portion of this liquid emulsion received no further treatment; to another portion was added one of the compounds described below. Both portions were coated on film support, and the dry films were exposed to red light in an intensity scale sensitometer. The exposed films were processed in reversal Color Process 1 and in the 5248 Negative Color Process 2 with the results shown in the following table. Color Process 2 was carried out as described by Hanson and Kisner JSMPT, 61, 667-701 (1953) for Color Negative Film, type 5248 involving the steps of color development,

The color developing solution above had the following composition:

|    |                                                                                              |        |       |
|----|----------------------------------------------------------------------------------------------|--------|-------|
| 55 | Water, 70 to 80° F. (21 to 27° C.)                                                           | liters | 1.0   |
|    | Benzyl alcohol                                                                               | cc     | 6.0   |
|    | Sodium hexametaphosphate                                                                     | grams  | 2.0   |
|    | Sodium sulfite, desiccated                                                                   | do     | 5.0   |
|    | Trisodium phosphate                                                                          | do     | 40.0  |
| 60 | Potassium bromide                                                                            | do     | 0.25  |
|    | 0.1% solution of potassium iodide                                                            | cc     | 10.0  |
|    | Sodium hydroxide                                                                             | grams  | 6.5   |
| 65 | (4 - amino - N - ethyl-N-[β-methanesulfonamidoethyl] m - toluidine sesquisulfate monohydrate | grams  | 11.33 |
|    | Ethylenediamine sulfate                                                                      | do     | 7.8   |
|    | Citrazinic acid (2,6 - dihydroxyisonicotinic acid)                                           | grams  | 1.5   |

The silver bleaching solution above had the following composition:

|    |                        |        |      |
|----|------------------------|--------|------|
| 70 | Water 90° F. (32° C.)  | liters | 1.0  |
|    | Potassium dichromate   | grams  | 5.0  |
|    | Potassium ferricyanide | do     | 70.0 |
| 75 | Potassium bromide      | do     | 20.0 |

The fixing baths above had the following composition:

|                        |        |       |
|------------------------|--------|-------|
| Water, 80° F. (27° C.) | liters | 1.0   |
| Sodium thiosulfate     | grams  | 150.0 |
| Sodium bisulfite       | do     | 20.0  |

TABLE VI

| Number | Feature                       | Color Process 1<br>(Reversal)<br>Speed Inc<br>(Log E) <sup>1</sup> | Color Process 2 (5248<br>Negative)<br>Speed Increase<br>(Log E) <sup>2</sup> | 10 |
|--------|-------------------------------|--------------------------------------------------------------------|------------------------------------------------------------------------------|----|
| 19360  | Control                       | +0.25                                                              | +0.24                                                                        |    |
| 19367  | Compound I 2.0 g./mole AgX    | +0.10                                                              | +0.16                                                                        |    |
| 19637  | Control                       | +0.10                                                              | +0.16                                                                        | 15 |
| 19640  | Compound III 2.0 g./mole AgX  | +0.16                                                              | +0.14                                                                        |    |
| 19242  | Control                       | +0.16                                                              | +0.14                                                                        |    |
| 19243  | Compound V 0.5 g./mole AgX    | +0.06                                                              | +0.04                                                                        |    |
| 17139  | Control                       | +0.16                                                              | +0.16                                                                        |    |
| 17140  | Compound XIII 2.0 g./mole AgX | +0.06                                                              | +0.04                                                                        |    |
| 19546  | Control                       | +0.16                                                              | +0.16                                                                        |    |
| 19558  | Compound XV 2.0 g./mole AgX   | +0.16                                                              | +0.16                                                                        |    |

<sup>1</sup> Determined by measuring the shift of the reversal dye curve on the log E axis at a given density below maximum density.

<sup>2</sup> Determined by measuring the shift of the negative dye curve on the log E axis at a given density above minimum density.

## EXAMPLE 7

A high-speed bromoiodide emulsion chemically sensitized with sulfur and gold compounds and optically sensitized with a cyanine dye was provided. To various samples of the emulsion were added the ingredients shown in the following table. Sensitometric evaluation of the samples was carried out as in Example 1 with the result shown in the table.

TABLE VII

| Number | Feature                                                                               | Speed | $\gamma$ | Fog | 35 |
|--------|---------------------------------------------------------------------------------------|-------|----------|-----|----|
| 1212   | Control                                                                               | 304   | 1.14     | .08 |    |
| 1214   | 4,11-Diaza-3,12-dioxotetradecane-1,14-bis(pyridinium perchlorate) (I) .75 g./mole AgX | 313   | 1.42     | .10 |    |
| 1216   | 2,13-Diaza-3,12-dioxotetradecane-1,14-bis(pyridinium chloride) (Ir) .75 g./mole AgX   | 310   | 1.26     | .10 | 40 |
| 1217   | 4-Hydroxy-6-methyl-1,3,3a,7-tetrazaindene (XXX) 3.0 g./mol AgX                        | 309   | 1.24     | .08 |    |
| 1218   | (XXX) 3.0 g./mol+(I) .75 g./mol AgX                                                   | 314   | 1.23     | .10 |    |
| 1219   | (XXX) 3.0 g./mol+(I) 3.0 g./mol AgX                                                   | 321   | 1.17     | .10 |    |
| 1222   | (XXX) 3.0 g./mol+(Ir) .75 g./mol AgX                                                  | 311   | 1.22     | .10 |    |
| 1223   | (XXX) 3.0 g./mol+(Ir) 3.0 g./mol AgX                                                  | 312   | 1.19     | .11 | 45 |

The data in the above table clearly show the superiority of the amide compound I to the "reverse" amide Ir as an emulsion sensitizing agent.

The bis-quaternary salts described above can be used in emulsions in the manner of the above examples in concentrations of the order of about 0.02 to 4 grams per mol of silver halide.

The emulsions may also be developed in the presence of the bis-quaternary salts by incorporating the salts into a developer solution. For example, when compound V was incorporated into the negative developer (2 g. per liter) of Color Process 1 of Example 6 and a multilayer color film containing couplers in the emulsion layers was developed therein, speed increases were obtained particularly for the green- and red-sensitive emulsion layers.

As indicated in the above examples, it may be desirable to incorporate a stabilizing agent into the emulsion sensitized with the bis-quaternary salts of the invention to reduce fog to normal levels. Azaindenes particularly suitable for this purpose are those described in the Carroll et al. U.S. patent application Serial Nos. 627,135 and 627,136, filed Dec. 10, 1956, for example, the following: 5-carboxy-4-hydroxy-1,3,3a,7-tetrazaindene; 1,2-bis(4-hydroxy-6-methyl-1,3,3a,7-tetrazaindene-5-yl)ethane; 1,2,3,4-tetrakis(4-hydroxy-6-methyl-1,3,3a,7-tetrazaindene-2-yl)butane; 2-amino-5-carboxy-4-hydroxy-1,3,3a,7-tetrazaindene; 4-hydroxy-6-methyl-1,3,3a,7-tetrazaindene; 4-hydroxy-2-β-hydroxyethyl-6-methyl-1,3,

3a, 7-tetrazaindene, 5-carboxy-4-hydroxy-1,3,3a,7-tetrazaindene; 7-hydroxy-1,2,3,4,6-pentazaindene; 2,4-dihydroxy-6-methyl-1,3,3a,7-tetrazaindene; 4-hydroxy-2-β-hydroxypropyl-6-methyl-1,3,3a,7-tetrazaindene and 4-hydroxy-2-(4-pyridyl)-6-methyl-1,3,3a,7-tetrazaindene.

The preparation of silver halide emulsions involves three separate operations: (1) the emulsification and digestion or ripening of the silver halide, (2) the freeing of the emulsion from aqueous soluble salts usually by washing, (3) the second digestion or after-ripening to obtain increased sensitivity (Mees, The Theory of the Photographic Process, 1942, page 3). The sensitizing agents may be added at any stage, preferably after the final digestion.

The photographic emulsions which we use are of the developing-out type and best results have been obtained with gelatino-silver bromoiodide emulsions. However, emulsions of varying silver halide content may be used.

The emulsions are chemically sensitized by any of the accepted procedures in addition to sensitizing with the bis-quaternary salts of the invention. The emulsions may be digested with naturally active gelatin, or sulfur compounds may be added such as those described in Sheppard U.S. Patents 1,574,944 and 1,623,499, and Sheppard and Brigham U.S. Patent 2,410,689.

The emulsions may also be treated with salts of the noble metals such as ruthenium, rhodium, palladium, iridium and platinum, all of which belong to group VIII of the periodic table of elements and have an atomic weight greater than 100. Representative compounds are ammonium chloropalladate, potassium chloroplatinate and sodium chloropalladite, which are used for sensitizing in amounts below that which produces any substantial fog inhibition, as described in Smith and Trivelli U.S. Patent 2,448,060, and as anti-foggants in higher amounts, as described in Trivelli and Smith U.S. Patents 2,566,245 and 2,566,263.

The emulsions may also be chemically sensitized with gold salts as described in Waller and Dodd U.S. Patent 2,399,083 or stabilized with gold salts as described in Damschroder U.S. Patent 2,597,856 and Yützy and Leermakers U.S. Patent 2,597,915. Suitable compounds are potassium chloroaurite, potassium aurithiocyanate, potassium chloroaurate, auric trichloride and 2-aurosulfonylbenzothiazole methochloride.

The emulsions may also be chemically sensitized with reducing agents such as stannous salts (Carroll U.S. Patent 2,487,850), polyamines such as diethylene triamine (Lowe and Jones U.S. Patent 2,518,698), polyamines such as spermine (Lowe and Allen U.S. Patent 2,521,925), or bis-(β-aminoethyl) sulfide and its water-soluble salts (Lowe and Jones U.S. Patent 2,521,926).

Other compounds useful for suppressing the fog level of the emulsion sensitized with the bis-quaternary compounds of the invention include the mercury compounds of Allen et al. U.S. Patent 2,728,663, Carroll and Murray U.S. Patent 2,728,664 and Leubner and Murray U.S. Patent 2,728,665 granted December 27, 1955; and the organic mercury compounds of Carroll et al. U.S. Patent 2,784,090 granted March 5, 1957.

The emulsions may also contain polyalkylene oxides and derivatives thereof such as the polyethylene glycols, in addition to the bis-quaternary compounds of the invention. Suitable polyalkylene oxides and polyalkylene oxide derivatives are described in Blake U.S. Patent 2,441,389, May 11, 1948; Blake et al. U.S. Patents 2,400,532, May 21, 1946, 2,423,549, July 8, 1947, and Jennings et al. U.S. Patent 2,577,127, December 4, 1951.

Other stabilizing agents may be added to the emulsions containing the bis-quaternary salts such as the metal inorganic salts of U.S. patent application Serial No. 493,047, filed March 8, 1955, by J. E. Jones.

The chemical sensitizing agents and other addenda which we have described may be used in various kinds of photographic emulsions, e.g., various silver salts may be

used as the sensitive salt such as silver bromide, silver iodide, silver chloride or mixed silver halides such as silver chlorobromide or silver bromoiodide.

The dispersing agent for the silver halide may be gelatin or other hydrophilic material such as collodion, albumin, cellulose derivatives or synthetic resins.

Since the coupler-containing emulsions sensitized as described with the bis-quaternary salts are adapted particularly for use in color photography, they will ordinarily comprise the emulsion layers of multilayer color films which emulsion layers are customarily differentially sensitized to the primary regions of the visible spectrum and contain coupler compounds producing dye images of colors complementary to the sensitivity of the emulsion layers. In a representative color film, one or more of the differentially sensitized emulsion layers may be sensitized with the bis-quaternary salts, and in a typical example emulsions sensitized to the red, green and blue regions of the spectrum are superimposed on the support in that order and contain cyan, magenta and yellow color-forming coupler compounds respectively. A yellow filter layer is advantageously interposed between the blue and green-sensitive emulsion layers.

Since the emulsion layers sensitized with the bis-quaternary salts of the invention may contain coupler compounds they can be readily processed by well known methods to yield color negatives directly or positive images by means of well known reversal processes. That is, after initial exposure of the emulsion to a subject a developer of the p-phenylene diamine type will produce a colored image negative in respect to the subject. Likewise, if development of the emulsion layer is first carried out with a non-color-forming developer followed by reversal exposure of the residual silver halide and then color development, a colored positive is obtained as described in the examples above.

The coupler compounds used in the emulsion layers sensitized with the bis-quaternary salts, are any of the well known compounds which combine with the oxidation product of primary aromatic amino (p-phenylene diamines) silver halide color developing agents to form dyes, for example, the phenolic couplers of U.S. Patents 2,266,452, 2,362,598, 2,589,004, 2,474,293, 2,521,908, 2,423,730 and Fierer U.S. patent application 476,561; the pyrazolone couplers of U.S. Patents 1,969,479, 2,369,489, 2,600,788, 2,618,641, 2,511,231 and the open chain reactive methylene couplers of U.S. Patents 2,298,443, 2,652,329, 2,407,210, 2,271,238 and McCrossen et al. U.S. patent application Serial No. 575,099, filed March 30, 1956. Likewise, the emulsions may contain colored color-forming couplers as described in U.S. Patents 2,521,908, 2,706,684, 2,455,169, 2,694,703, 2,455,170 and 2,453,661.

The couplers may be dispersed in the emulsion layers by means of an oily coupler solvent according to the methods of U.S. Patents 2,304,940 and 2,322,027. However, if as may be the case, the couplers contain solubilizing groups such as  $\text{SO}_3\text{H}$  groups which render the couplers soluble in alkaline solution, the oily coupler solvent may be dispensed with and the couplers can be added to the emulsion from aqueous solutions as their alkali metal salts.

What we claim is:

1. A photographic silver halide emulsion containing a quaternary ammonium salt having a general formula of the class consisting of



and



wherein Q and Q' each represent radicals of the class 70 consisting of



wherein  $\text{R}^2$ ,  $\text{R}^3$  and  $\text{R}^4$  represent lower alkyl groups, Z represents the atoms necessary to complete a heterocyclic nucleus of the class consisting of pyridinium and quinolinium, R and R' each represent alkylene groups linked directly to the quaternary nitrogen atoms of said radicals, n represents a positive integer of from 1 to 2, A represents a member of the class consisting of



20



and



25

30

wherein  $n'$  and  $n''$  represent positive integers of from about 1 to 10 there being from about 14 to about 30 atoms present in the shortest linear chain of atoms linking said quaternary nitrogen atoms.

2. A photographic silver halide emulsion containing a quaternary ammonium salt having the general formula



wherein Q and Q' each represent radicals of the class consisting of



wherein  $\text{R}^2$ ,  $\text{R}^3$ , and  $\text{R}^4$  represent lower alkyl groups, Z represents the atoms necessary to complete a heterocyclic nucleus of the class consisting of pyridinium and quinolinium, R and R' each represent alkylene groups linked directly to the quaternary nitrogen atoms of said radicals, n represents a positive integer of from 1 to 2, A represents a member of the class consisting of



50



55

60

65

and



65

70

75

wherein  $n'$  and  $n''$  represent positive integers of from about 1 to 10, there being from 14 to about 30 atoms present in the shortest linear chain of atoms linking said quaternary nitrogen atoms.

19

3. A photographic silver halide emulsion containing a quaternary ammonium salt having the general formula



wherein Q and Q' each represent radicals of the class consisting of



wherein R<sup>2</sup>, R<sup>3</sup>, and R<sup>4</sup> represent lower alkyl groups, Z represents the atoms necessary to complete a heterocyclic nucleus of the class consisting of pyridinium and quinolinium, R and R' each represent alkylene groups linked directly to the quaternary nitrogen atoms of said radicals, A represents an alkylene group of from about 1 to 10 carbon atoms, there being from about 14 to about 30 atoms present in the shortest linear chain of atoms linking said quaternary nitrogen atoms.

4. A photographic silver halide emulsion containing the compound 7,14-diaza-6,15-dioxoecosane - 1,20 - bis(pyridinium perchlorate).

5. A photographic silver halide emulsion containing the compound 7,18-diaza-6,19-dioxotetracosane - 1,24 - bis(pyridinium perchlorate).

6. A photographic silver halide emulsion containing the compound 10,15-diaza-9,16-dioxotetracosane-1,24-bis(pyridinium perchlorate).

7. A photographic silver halide emulsion containing the compound 12,15-diaza-11,16 - dioxohexacosane - 1,26- bis(pyridinium perchlorate).

8. A photographic silver halide emulsion containing the compound 12,19-diaza - 11,20 - dioxotriacontane-1,30- bis(pyridinium perchlorate).

9. The emulsion of claim 1 further containing a coupler compound reactive with the oxidation products of a p-phenylene diamine silver halide developing agent to form a dye.

10. The emulsion of claim 2 further containing a coupler compound reactive with the oxidation products of a p-phenylene diamine silver halide developing agent to form a dye.

11. The emulsion of claim 3 further containing a coupler compound reactive with the oxidation products of a p-phenylene diamine silver halide developing agent to form a dye.

12. The emulsion of claim 1 further containing an azaindene stabilizing agent.

13. The emulsion of claim 2 further containing an azaindene stabilizing agent.

14. The emulsion of claim 2 further containing an azaindene stabilizing agent.

15. The emulsion of claim 1 wherein the silver halide is sulfur and gold sensitized.

16. A method for increasing the speed of a silver halide

20

emulsion which comprises developing said emulsion in the presence of a quaternary ammonium salt having a general formula of the class consisting of



and



wherein Q and Q' each represent radicals of the class consisting of



wherein R<sup>2</sup>, R<sup>3</sup>, and R<sup>4</sup> represent lower alkyl groups, Z represents the atoms necessary to complete a heterocyclic nucleus of the class consisting of pyridinium and quinolinium, R and R' each represent alkylene groups linked directly to the quaternary nitrogen atoms of said radicals, n represents a positive integer of from 1 to 2, A represents a member of the class consisting of



wherein n' and n'' represent positive integers of from about 1 to 10, there being from about 14 to about 30 atoms present in the shortest linear chain of atoms linking said quaternary nitrogen atoms.

#### References Cited in the file of this patent

##### UNITED STATES PATENTS

- 2,288,226 Carroll et al. June 30, 1942  
 2,419,975 Trivelli et al. May 16, 1947  
 2,784,090 Carroll Mar. 5, 1957

##### FOREIGN PATENTS

- 115,971 Australia Oct. 15, 1942

UNITED STATES PATENT OFFICE  
CERTIFICATE OF CORRECTION

Patent No. 2,940,851

June 14, 1960

Dorothy J. Beavers et al.

It is hereby certified that error appears in the printed specification of the above numbered patent requiring correction and that the said Letters Patent should read as corrected below.

Column 1, line 27, for "emulsions," read -- emulsions. --; column 18, line 18, for that portion of the formula reading "-(CH<sub>2</sub>)<sub>n</sub>-" read -- -(CH<sub>2</sub>)<sub>n</sub>'- --; column 19, line 51, for the claim reference numeral "2" read -- 3 --; column 20, line 30, for that portion of the formula reading "-(CH<sub>2</sub>)<sub>n</sub>-" read -- -(CH<sub>2</sub>)<sub>n</sub>'- --.

Signed and sealed this 11th day of April 1961.

(SEAL)

Attest:

ERNEST W. SWIDER  
Attesting Officer

ARTHUR W. CROCKER  
Acting Commissioner of Patents